

UNITED STATES PATENT OFFICE

2.577.127

# PHOTOGRAPHIC ELEMENT WITH COLLOID LAYER CONTAINING COLOR FORMER AND NONIONIC WETTING AGENT

**Andrew Bradshaw Jennings, Edgebrook, and Otis Willard Murray, Rumson Park, N. J., assignors to E. I. du Pont de Nemours & Company, Wilmington, Del., a corporation of Delaware**

**No Drawing. Application November 23, 1946,  
Serial No. 711,836**

9 Claims. (Cl. 95—7)

1

This invention relates to color photography. More particularly, it relates to color-forming silver halide emulsions and emulsion layers containing non-ionic wetting agents. It also relates to photographic elements containing such emulsion layers.

It has been proposed to add various wetting agents of the ionic type to photographic silver halide emulsions with high molecular weight color formers in order to facilitate dispersion of the latter. The wetting agents so proposed have the objection that they leave a colored stain in the emulsion layers after development and removal of the silver images and silver salts. This stain results in a multicolor picture which has improper color values and is not an accurate reproduction.

An object of the present invention is to improve the chromogenic development of silver halide images. A further object is to eliminate the stain in prior art procedures utilizing wetting agents. Another object is to provide photographic emulsion layers which can be color developed and washed without producing objectionable color stain. Still other objects will be apparent from the following description of the invention.

It has been found that the addition of non-ionic wetting agents to photographic silver halide emulsion layers prior to development thereof is advantageous in the color development thereof. It is especially true of such development when high molecular weight or non-diffusing color formers or polymeric color formers are present in the emulsion layers. Such agents are preferably added to the photographic silver halide emulsions prior to the addition of the color formers thereto because they assist in the dispersion of the color formers in such emulsions.

Various types of non-ionic wetting agents are known. In general, they are free from sulfonic acid and carboxylic acid groups and quaternary nitrogen salt groups and contain a plurality of oxygen atoms. A class of especially useful products have a structure which is exemplified by the following hexitans and hexide derivative formulae

## ANSWER



$$\begin{array}{c}
 (3) \quad \text{O} \\
 \text{R}-\text{C}-\text{C}-\text{CH}_2 \\
 | \quad | \quad | \\
 \text{H}_2\text{C} \quad \text{C}-\text{CH}-\text{O}-(\text{Alkylene}-\text{O})_n-\text{R}
 \end{array}$$

wherein in the formulae one of the R's is an alkyl radical of 8 to 20 carbon atoms or an acyl radical of the formula, R—CO— wherein R has the same value and the other R's are hydrogen and n is 2 to 30 or more.

Another class of useful compounds consists of the higher polyglycols having an average molecular weight of at least 400 and especially those having a molecular weight or average molecular weight of at least 1500.

The polyglycols described above are known chemical compounds and many of them are available commercially. They can be prepared in various ways; for example, by the removal of water from glycols and by the reaction of oxides with glycols. The reactions are generally carried out until the products have a molecular weight or an average molecular weight in excess of 400. Ethylene oxide, propylene oxide-1,2, and -1,3 and butylene oxides-1,2 can be used in the preparation of the products and they may be reacted with ethylene glycol, diethylene glycol. Their preparation is described in *The Chemistry of Synthetic Resins*, pages 990-994 published by Rheinhold Publishing Corp. (1935).

Preferred compounds of this type may be represented by the formula



40 where  $n$  is 7 to 200 or more. Compounds having such a formula include nonaethylene glycol, decaethylene glycol, dodecaethylene glycol and higher homologues containing from 9 to 200  $-\text{CH}_2\text{CH}_2\text{O}-$  groups. The lower members of  
45 the class are viscous liquids to semi-solids and solids, at 20° C., which are somewhat hygroscopic up to a molecular weight in excess of 1500. The higher homologues are waxy solids and as their  
50 molecular weight increases to 4000 they become non-hygroscopic in character. The lower members of the series are easily soluble in water, the solubility becoming less as the molecular weights of the compound increase. In general, the higher  
55 members of the series cannot be too easily isolated as single chemical entities. Instead, the

condensation reaction leading to their preparation is carried to a point where the bulk of the material will consist of homologous compounds of similar chain length. Mixtures of two or more polyalkylene glycols or polyoxyalkylene glycols are selected on the basis of average molecular weight. Since a difference of one or two ethylene oxide links in polymers of considerable chain length has a negligible effect on their physical and chemical properties, such mixtures can be readily employed in the present invention. For the purposes of this invention, it is sufficient to know the average molecular weight of the material to be used and the fact that it may in all likelihood consist of a mixture of several compounds of closely similar molecular weights does not reduce its effectiveness.

The lower alkyl ethers and carboxylic acid esters of the aforesaid polyglycols are also useful. Among such ethers and esters are the mono- and di-methyl and mono- and di-ethyl ethers and the mono- and di-acetates, formates, and propionates.

Still other useful compounds are disclosed in Meincke United States Patent 2,341,846 which are free from free sulfonic and carboxylic acid or their salt groups. Yet others are disclosed in Swan United States Patent 2,240,472.

The compounds are preferably admixed with the silver halide colloid emulsions prior to the addition of the color formers. This may be accomplished by means of water or water-solvent mixtures, e. g., methyl alcohol, ethyl alcohol, and acetone, containing the non-ionic wetting agents. The color formers can be added from the same solution or separately. After addition of the color former and wetting agent, the solution is brought to a proper viscosity for coating. The non-ionic wetting agents may be used over a wide range of proportions. A practical range is 0.1 gram to 2.0 grams per liter of colloid silver halide emulsion.

Various types of hydroscopic wetting agents may be used in conjunction with the non-ionic wetting agents if desired. They eliminate or remove any stain produced by ionic wetting agents upon an adequate washing of the color developed elements.

The non-ionic wetting agents aid in coating of color-forming photographic colloid silver halide emulsion layers and prevent coating streaks, repellent spots and bubble formation. In addition, they permit satisfactory rewetting of the dried layers.

The invention will be further illustrated by the following examples.

#### Example I

To 250 grams of a negative type, flowable, gelatino-silver iodobromide emulsion is added one gram of 4,4'-methylene-bis-(1-phenyl-3-methyl-5-pyrazolone). Two cubic centimeters of a 10% aqueous solution of a mannitan monolaurate containing 2 to 3 polyoxyethylene chains of 8 or more carbon atoms is added. The resulting emulsion is coated onto a cellulose acetate film base and dried. The film element is exposed to form an image record and then developed in a solution of the following composition:

|                                       |        |      |
|---------------------------------------|--------|------|
| N-p-diethylaminoaniline hydrochloride | grams  | 3.0  |
| Sodium carbonate (anhydrous)          | grams  | 25.0 |
| Potassium bromide                     | grams  | 1.5  |
| Sodium sulfite (anhydrous)            | grams  | 7.0  |
| Water to                              | liters | 1.0  |

A similar emulsion is prepared by substituting sodium dodecylsulfate for the mannitan derivative and coated and the resulting element exposed and processed in like manner. The two developed elements are then bleached in potassium ferricyanine and fixed in sodium thiosulfate. In each case the highlight density was measured to determine the amount of stain present. The latter element has 50% more stain when measured by a densitometer than the former. There was no evidence of differences in black and white fog on the two films.

Similar results are obtained by adding 12 cc. of 5% saponin solution to the emulsions prior to coating.

#### Example II

A cellulose acetate film base is coated with an 8% aqueous gelatin solution containing one gram of 4,4'-bis-(1-naphthol-2-sulfamidophenyl) ether, 10 cc. of 5% aqueous saponin solution, and 1 cc. of the mannitan derivative of Example I per 100 cc. of gelatin solution to form a thin, color-yielding substratum. A gelatino-silver iodobromide emulsion containing 8 cc. of 5% saponin solution and 1% of the same mannitan monolaurate derivative per 100 cc. of wet emulsion is coated onto said substratum.

A similar element is made by substituting for the non-ionic wetting agent similar amounts of sodium dodecyl sulfate.

The two elements just described are exposed to an object and developed, bleached, fixed, and washed as in Example I. The first element is practically free from color stain, whereas the latter has a significant color stain.

The elements are not limited to the particular film elements described above. Thus single and multilayer elements on various types of supports, e. g., paper, metal, superpolymers, e. g., nylon 40 polystyrene, polymerized methyl methacrylate, polyvinyl chloride; cellulose nitrate, cellulose acetate propionate, cellulose acetate butyrate, etc. may be made. Multilayer elements containing, for example, different color formers and the same 45 or different non-ionic wetting agents can be made in like manner by coating the color-yielding emulsions onto the support or a coated layer superposed thereon.

In place of the specific color formers described 50 in the examples, there may be substituted other such materials. Among the useful ones are those described in United States Patents 2,294,909, 2,368,302, 2,395,484, 2,397,864, 2,397,865, 2,397,867, 2,319,426, 2,299,641 and 2,283,276.

In place of the saponin of the above examples, 55 there may be substituted various other hydroscopic agents. Suitable additional ones include alkali metal salts of alkylated naphthalene sulfonic acids, alkali metal salts of long chain alkyl sulfates and alkyl sulfonates. Still other hydroscopic agents are described in Ullman Encyclopaedie der Technischen Chemie, 2nd edition, vol. IX, page 808. The agents may be used over a fairly wide range. For example, they may be used in the water-permeable layers, both of the light-sensitive and light-insensitive type, in an amount from 0.05 to 1% or more, based on the solids in solution.

An advantage of the invention is that it provides a simple and economical method of removing color stain from photographic elements. A further advantage is that the agents improve the rewetting characteristics of a water-permeable colloid layer resulting in a uniformity of results.

As many widely different embodiments of this

Invention can be made without departing from the spirit and scope thereof, it is to be understood that the invention is not to be limited except as defined by the claims.

What is claimed is:

1. A photographic element bearing a light sensitive silver halide stratum and at least one water-permeable colloid layer containing a color former containing as an active color-coupling group a structure of the formula



where  $X$  is a member of the group consisting of  $-OH$  and  $-NHR$ , where  $R$  is a member of the group consisting of  $H$  and aliphatic hydrocarbon radicals, said color former being capable of forming a dye taken from the group consisting of quinoneimine and azomethine dyes and a non-ionic wetting agent having a molecular weight of at least 400, and a plurality of oxyalkylene groups in a chain of atoms, said agent being free from sulfonic and carboxylic acid and quaternary nitrogen salt groups.

2. A photographic element bearing a light-sensitive silver halide stratum and at least one gelatin layer containing a color former containing as an active color-coupling group a structure of the formula



where  $X$  is a member of the group consisting of  $-OH$  and  $-NHR$ , where  $R$  is a member of the group consisting of  $H$  and aliphatic hydrocarbon radicals, said color former being capable of forming a dye taken from the group consisting of quinoneimine and azomethine dyes and a non-ionic wetting agent having a molecular weight of at least 400, and a plurality of oxyalkylene groups in a chain of atoms, said agent being free from sulfonic and carboxylic acid and quaternary nitrogen salt groups.

3. A photographic element bearing a light-sensitive silver halide stratum and at least one water-permeable colloid layer containing a color former containing as an active color-coupling group a structure of the formula



where  $X$  is a member of the group consisting of  $-OH$  and  $-NHR$ , where  $R$  is a member of the group consisting of  $H$  and aliphatic hydrocarbon radicals, said color former being capable of forming a dye taken from the group consisting of quinoneimine and azomethine dyes, light-sensitive silver halides, and a non-ionic wetting agent having a molecular weight of at least 400, and a plurality of oxyalkylene groups in a chain of atoms, said agent being free from sulfonic and carboxylic acid and quaternary nitrogen salt groups.

4. A photographic element bearing at least one gelatin layer containing a color former containing as an active color-coupling group a structure of the formula



where  $X$  is a member of the group consisting of  $-OH$  and  $-NHR$ , where  $R$  is a member of the group consisting of  $H$  and aliphatic hydrocarbon radicals, said color former being capable of forming a dye taken from the group consisting of quinoneimine and azomethine dyes, light-sen-

sitive silver halides, and a non-ionic wetting agent having a molecular weight of at least 400, and a plurality of oxyalkylene groups in a chain of atoms, said agent being free from sulfonic and carboxylic acid and quaternary nitrogen salt groups.

5. A photographic element bearing a light sensitive silver halide stratum and at least one water-permeable colloid layer containing a color former containing as an active color-coupling group a structure of the formula



15 where  $X$  is a member of the group consisting of  $-OH$  and  $-NHR$ , where  $R$  is a member of the group consisting of  $H$  and aliphatic hydrocarbon radicals, said color former being capable of forming a dye taken from the group consisting of quinoneimine and azomethine dyes, a non-ionic wetting agent having a molecular weight of at least 400, and a plurality of oxyalkylene groups in a chain of atoms, said agent being free from sulfonic and carboxylic acid and quaternary nitrogen salt groups, and a hydroscopic wetting agent.

20 6. The process of reducing color stain which comprises developing a photographic element containing a color former containing as an active color-coupling group a structure of the formula



35 where  $X$  is a member of the group consisting of  $-OH$  and  $-NHR$ , where  $R$  is a member of the group consisting of  $H$  and aliphatic hydrocarbon radicals, said color former being capable of forming a dye taken from the group consisting of

40 quinoneimine and azomethine dyes and a silver halide image in the presence of a non-ionic wetting agent having a molecular weight of at least 400, and a plurality of oxyalkylene groups in a chain of atoms, said agent being free from sulfonic and carboxylic acid and quaternary nitrogen salt groups and removing the silver and silver salts.

45 7. A photographic element bearing at least one water-permeable colloid layer containing a color former containing as an active color-coupling group a structure of the formula



55 where  $X$  is a member of the group consisting of  $-OH$  and  $-NHR$ , where  $R$  is a member of the group consisting of  $H$  and aliphatic hydrocarbon radicals, said color former being capable of forming a dye taken from the group consisting of quinoneimine and azomethine dyes, light-sensitive silver halides, and from 0.1 to 2.0 grams per liter of emulsion of a polyethylene glycol containing from 7 to 200  $-CH_2CH_2O-$  groups.

60 8. A photographic element bearing at least one gelatin layer containing 4,4'-methylene-bis-(1-phenyl-3-methyl-5-pyrazolone), light-sensitive silver halides, and from 0.1 to 2.0 grams per liter of emulsion of a mannan monolaurite containing 2 to 3 polyoxyethylene chains of at least 8 carbon atoms.

65 9. A photographic element bearing at least one gelatin layer containing 4,4'-bis-(1-naphthyl-2-sulfamido phenyl)ether, light-sensitive silver halides, and from 0.1 to 2.0 grams per liter of emulsion of a mannan monolaurite containing

2 to 3 polyoxyethylene chains of at least 8 carbon atoms.

ANDREW BRADSHAW JENNINGS,  
OTIS WILLARD MURRAY.

REFERENCES CITED

The following references are of record in the file of this patent:

UNITED STATES PATENTS

|           |               |              |
|-----------|---------------|--------------|
| Number    | Name          | Date         |
| 2,186,717 | Eggert et al. | Jan. 9, 1940 |

| Number      | Name            | Date          |
|-------------|-----------------|---------------|
| 2,240,472   | Swan            | Apr. 29, 1941 |
| 2,304,940   | Mannes et al.   | Dec. 15, 1942 |
| 2,322,027   | Jelley et al.   | June 15, 1943 |
| 5 2,324,831 | Frohlich et al. | July 20, 1943 |
| 2,353,262   | Peterson et al. | July 11, 1944 |
| 2,360,290   | Vittum et al.   | Oct. 10, 1944 |
| 2,423,549   | Blake et al.    | July 8, 1947  |

10 FOREIGN PATENTS

|         |               |              |
|---------|---------------|--------------|
| Number  | Country       | Date         |
| 442,522 | Great Britain | Feb. 3, 1936 |